

G. P. HULST.

PROCESS OF REFINING AND DESILVERIZING LEAD.

APPLICATION FILED OCT. 28, 1910.

1,001,525.

Patented Aug. 22, 1911.

3 SHEETS-SHEET 1.



Johns B. Bunting  
R. J. Foster

INVENTOR  
George P. Hulst  
Munro & Co.  
ATTORNEYS

G. P. HULST.

PROCESS OF REFINING AND DESILVERIZING LEAD.

APPLICATION FILED OCT. 28, 1910.

1,001,525.

Patented Aug. 22, 1911.

3 SHEETS—SHEET 2.



WITNESSES

John Bergman  
H. F. Hartley

INVENTOR

George P. Hulst  
BY *Munroes.*

ATTORNEYS

G. P. HULST.

PROCESS OF REFINING AND DESILVERIZING LEAD.

APPLICATION FILED OCT. 28, 1910.

1,001,525.

Patented Aug. 22, 1911.

3 SHEETS—SHEET 3.



Fig. 4

WITNESSES

John A. Scovron  
Rev. F. Koester, Jr.

INVENTOR

George P. Hulst  
BY *Maurand Co.*

ATTORNEYS

# UNITED STATES PATENT OFFICE.

GEORGE P. HULST, OF OMAHA, NEBRASKA.

## PROCESS OF REFINING AND DESILVERIZING LEAD.

1,001,525.

Specification of Letters Patent. Patented Aug. 22, 1911.

Application filed October 28, 1910. Serial No. 589,589.

To all whom it may concern:

Be it known that I, GEORGE P. HULST, a citizen of the United States, and a resident of Omaha, in the county of Douglas and State of Nebraska, have invented a new and Improved Process of Refining and Desilverizing Lead, of which the following is a full, clear, and exact description.

The invention relates to refining and desilverizing by the crystallization process, and its object is to provide a new and improved method for refining and desilverizing lead bullion and impure lead, and whereby the number of crystallizing operations is reduced to a minimum for the proper production of high grade bullion or metal running five hundred to six hundred ounces silver and a market lead.

The invention consists in a method whereby the crystals in a crystallizing kettle are subjected to pressure to squeeze out the uncryallized liquid.

In order to carry out this method, use is made of an apparatus, such, for instance, as shown in the accompanying drawings forming a part of this specification, in which similar characters of reference indicate corresponding parts in all the views.

Figure 1 is a side elevation of a series of six kettles and the framework and overhead crane used in lifting the kettles and the press; Fig. 2 is an enlarged sectional side elevation of one of the kettles and the press in position thereon; Fig. 3 is a side elevation of the upper end of one of the kettles and the lower ends of the standards of the press fastened in place on the kettle; and Fig. 4 is an enlarged sectional side elevation of one of the kettles in which a fluid under pressure is used for squeezing out the uncryallized liquid.

The crystallization processes heretofore used are based on the fact that lead or lead bullion carrying silver, gold, and other impurities, such as bismuth, copper, arsenic, zinc, antimony, and the like, and cooled down to nearly a solidifying point and stirred by hand or mechanically by suitable devices in a crystallizing kettle, form crystals of lead which are freer from silver and other impurities, such as above mentioned, than the liquid which permeates the entire mass of mushy crystals.

In the crystallization process referred to the uncryallized liquid is strained off by gravity through one or more tap holes in the

bottom of the crystallizing kettle, and it takes usually about twelve crystallization operations to produce market lead at one end and five hundred ounces per ton metals for cupeling at the other end. The crystals are granular and spongy, and a quantity of uncryallized lead or liquid is held in suspension or permeates the whole mass of crystals, and by gravity not all of this uncryallized lead is strained out in the processes mentioned and heretofore used. With my invention, presently to be described in detail, the crystals are subjected to pressure so as to squeeze out the uncryallized lead or liquid from the crystals to render the latter drier, that is, freer from the liquid lead, which latter is higher in silver and other impurities than the crystals. With my improvement the number of kettles and the number of crystallizing operations are reduced to about six, that is, one-half of that heretofore required, and hence a direct output of market lead can be obtained in a comparatively short time.

A series of kettles A, A', A<sup>2</sup>, A<sup>3</sup>, A<sup>4</sup> and A<sup>5</sup> are placed apart and arranged preferably as shown in Fig. 1, and each kettle is adapted to be raised to permit of running the molten liquid from a raised kettle into a lower non-raised kettle, as hereinafter more fully explained. Each kettle is enclosed in a shell B and is provided with a valved outlet or spout C adapted to be connected by a trough C' with another kettle, as indicated in Fig. 1.

Into each of the kettles opens at the bottom a steam supply pipe D directly under a baffle plate E, as plainly shown in Fig. 2, so that steam can be passed into the molten lead with a view to cool the same and to cause agitation thereof for the formation of the crystals, as is well known in the crystallization process. Each of the steam supply pipes D is provided with a valve D' for controlling the steam passing into the corresponding kettle, and each steam supply pipe D has a sliding connection with a fixed pipe D<sup>2</sup> (see Fig. 1), connected with a boiler or other suitable source of steam supply.

Under each kettle is arranged a burner F having a pipe F' provided with a valve F<sup>2</sup>, the said pipe F' having a sliding connection with a supply pipe F<sup>3</sup> connected with a suitable source of gas supply, so that the kettle may be heated whenever it is desired to do so.

The top of each kettle A, A', A<sup>2</sup>, A<sup>3</sup>, A<sup>4</sup> and A<sup>5</sup> is provided with sets of lugs G, on which are removably fastened by keys G' the lower ends of standards H' of a press 5 H, having a cylinder H<sup>2</sup> mounted to slide up and down on the standards H'. In the cylinder H<sup>2</sup> is arranged a piston I attached to rods I' extending upwardly and secured to a top plate J carried by the standards H'. 10 On the lower end of the cylinder H<sup>2</sup> is secured a presser plate K adapted to pass into the corresponding kettle with which the press H is connected at the time, so as to subject the crystals therein to pressure with 15 a view to squeeze out of the crystals the uncrystallized liquid, as hereinafter more fully explained. A pipe L connected with an elastic fluid pressure supply opens into the lower end of the cylinder H<sup>2</sup>, and the 20 pipe L is provided with a three way valve L', which when turned one way allows the fluid pressure to pass into the lower end of the cylinder H<sup>2</sup>, to force the latter downward, thus moving the presser plate K into 25 the corresponding kettle for the purpose mentioned. When the valve L' is turned in the opposite direction it serves as an exhaust valve for the interior of the cylinder H<sup>2</sup>. A pipe N having a three way valve N' similar to the valve L' in the pipe L and also connected with a pressure supply opens into the upper end of the cylinder H<sup>2</sup>, to force the cylinder H<sup>2</sup> upward after the pressing 30 operation is completed. It will be understood that when one of the valves L' or N' is turned to its exhaust position the other valve is opened to admit fluid pressure into the cylinder.

The presser plate K is provided with 40 perforations K', and at one side with a depending channel K<sup>2</sup>, registering with a pipe K<sup>3</sup> fastened to the wall of the kettle (see Fig. 2), and provided with a valve K<sup>4</sup>. Now when the presser plate K moves downward in a kettle, the liquid passes up through the perforations K' onto the upper face of the presser plate K, to then run to the channel K<sup>2</sup> and out of the same by way of the now open pipe K<sup>3</sup> into a ladle or 45 into another kettle, as hereinafter more fully explained.

The top plate J of the press H is provided with a chain or loop O adapted to be connected with one of the hooks P' of an 50 overhead traveling crane P of any improved construction, to permit of raising and lowering the press H and to allow of bringing the press H into position on any one of the kettles A, A', A<sup>2</sup>, A<sup>3</sup>, A<sup>4</sup> and A<sup>5</sup>. It is 55 understood that when the press H has been lowered onto the top of any one of the kettles, it is readily fastened to the lugs G of this particular kettle by the keys G', so as to hold the press H temporarily in place on 60 the corresponding kettle. After the press-

ing operation is finished the keys G' are removed and the press H is lifted to disconnect it from the kettle and to allow of connecting the press with another kettle in which the next pressing operation is to take 70 place.

The kettles A, A', A<sup>2</sup>, A<sup>3</sup>, A<sup>4</sup> and A<sup>5</sup> are mounted to slide up and down in suitable guideways R (see Fig. 1) and each kettle is provided at its upper end with outwardly 75 extending lugs S. Disposed above the series of kettles is an overhead crane P provided with hooks P' arranged to engage a link T<sup>2</sup> of a cross head T', the latter is provided with a series of depending links T adapted to engage the lugs S in order to raise the kettles into their upper positions. It will be understood that as many of these lifting devices, similar to the ones just described, may be used as are necessary. 80

Now, by the arrangement described, any one of the kettles can be connected by the lifting device described with a hook P' of the overhead crane to raise this kettle into a discharging position, as indicated in Fig. 90 1, in which the kettles A, A<sup>2</sup> and A<sup>4</sup> are shown raised and connected by the troughs C' with the kettles A', A<sup>3</sup> and A<sup>5</sup>, appearing in lowermost position. The raised kettles are supported in the raised position 95 by suitable legs or props R', which are set under the kettles after they are raised.

The operation is as follows: When the apparatus is in use, alternate kettles are full while others are empty, the molten bullion 100 assaying in the several kettles when full as follows: The liquid high grade metal taken from the kettle A by way of the pipe K<sup>3</sup> assays 500 ounces Ag. per ton, the metal in the several kettles A, A', A<sup>2</sup>, A<sup>3</sup>, A<sup>4</sup> and A<sup>5</sup> 105 assaying per ton, respectively, 300 oz. Ag., 180 oz. Ag., 90 oz. Ag., 25 oz. Ag., 5 oz. Ag. and 1 oz. Ag., while the market lead from melted crystals in the kettle A<sup>5</sup> assays  $\frac{1}{10}$  oz. Ag. per ton. Presuming that the kettles A, 110 A<sup>2</sup> and A<sup>4</sup> are full of molten bullion of the grades above mentioned, while the kettles A' and A<sup>3</sup> are empty and the kettle A<sup>5</sup> is one-eighth (1/8) full from a previous operation, only tapping out six-eighths (6/8) 115 of market lead, so that the kettle A<sup>5</sup> fills from the kettle A<sup>4</sup> at the next operation and melted crystals run down. Presuming further that the apparatus is running seven-eighths (7/8) crystals, then the kettles A, A<sup>2</sup> 120 and A<sup>4</sup> are first allowed to cool down, the heat from the burners F being turned off, and then steam is admitted by way of the pipes D to form seven-eighths (7/8) crystals. This process can be hastened by supplying 125 water to the top of the lead through a pipe, the steam being temporarily shut off for the time. After the crystals are formed, the steam is shut off by closing the valves D'. A slow fire is now started under the kettles 130

A, A<sup>2</sup> and A<sup>4</sup> by the use of the burners F, and the said kettles are then raised by the use of the lifting device (T, T', T<sup>2</sup>) and overhead crane P to the position shown in 5 Fig. 1, and then the presses H are connected with the said kettles and set in action. The high grade metal pressed out in the kettle A is passed by way of its pipe K<sup>3</sup> into a ladle carried by the overhead crane P to 10 cupels, and the liquid pressed out in the kettle A<sup>2</sup> is passed by way of its pipe K<sup>3</sup> and a trough K<sup>5</sup> into the kettle A', while the pressed out liquid from the kettle A<sup>4</sup> is passed by way of its pipe K<sup>3</sup> and a trough 15 K<sup>6</sup> into the kettle A<sup>3</sup>. After one-eighth (1/8) liquid has been pressed out of the kettles A, A<sup>2</sup> and A<sup>4</sup>, more heat is turned on by the use of the burners F, to melt down the 20 pressed crystals. The presses H are now detached from the kettles A, A<sup>2</sup> and A<sup>4</sup>, and removed by the use of the overhead crane P. As soon as the crystals are melted down in 25 the kettles A, A<sup>2</sup> and A<sup>4</sup>, the valves in the outlets C for the said kettles are opened and the molten crystals from the kettle A are run into the kettle A', those from the kettle A<sup>2</sup> are run into the kettle A<sup>3</sup> and those from the kettle A<sup>4</sup> are run into the kettle A<sup>5</sup>, by way of the troughs C'. The 30 kettles A, A<sup>2</sup> and A<sup>4</sup> are now empty and are lowered to the level of the other kettles A', A<sup>3</sup> and A<sup>5</sup>, which are now full. It is understood that during the crystallizing of the lead by means of the steam and the subsequent melting down of the crystals, and 35 the transfer of the resulting liquid from one kettle to another various impurities are formed, and these drosses are skimmed off clean from the full kettles just before beginning the crystallization. The above-described operation relating to the kettles A, A<sup>2</sup> and A<sup>4</sup> is now repeated relative to the kettles A', A<sup>3</sup> and A<sup>5</sup>, that is, dry steam is turned on for the kettles A', A<sup>3</sup> and A<sup>5</sup>, to 40 crystallize their contents to seven-eighths (7/8), and then a slow fire is started under the said kettles A', A<sup>3</sup>, A<sup>5</sup> by the corresponding burners F, after which the kettles A', A<sup>3</sup>, A<sup>5</sup> are raised by the use of the overhead crane 45 P and supported by the legs R' in the raised position as before explained. The presses H are now applied to the raised kettles A', A<sup>3</sup>, A<sup>5</sup>, and actuated to press out the liquid and conduct the same by way of the corresponding pipes K<sup>3</sup> and troughs to the non-raised kettles A, A<sup>2</sup> and A<sup>4</sup>, that is, the liquid is run from kettle A' into kettle A, from kettle A<sup>3</sup> into kettle A<sup>2</sup> and from kettle A<sup>5</sup> into kettle A<sup>4</sup>. The burners F for 50 the kettles A', A<sup>3</sup> and A<sup>5</sup> are now turned on full, to melt down the crystals contained in the said kettles, after which the presses H are removed. The melted crystals from kettle A' are now run into kettle A<sup>2</sup>, and 55 those from kettle A<sup>3</sup> are run into kettle A<sup>4</sup> 60 and those from kettle A<sup>5</sup> are run into kettle A<sup>4</sup>.

by way of the outlets C and troughs C'. The kettles A', A<sup>3</sup>, and A<sup>5</sup> are now lowered and six-eighths (6/8) market lead is run off from the kettle A<sup>5</sup> into suitable molds. The other one-eighth (1/8) crystals are left in 70 the kettle A<sup>5</sup> so that the kettle A<sup>5</sup> is again filled with melted crystals at the next operation from the kettle A<sup>4</sup>, as previously explained. It will be noted that the kettle A is one-eighth (1/8) full while the kettles A<sup>2</sup>, 75 A<sup>4</sup> are completely filled and crystals are in each kettle and high grade metal and market lead has been run off. Seven-eighths (7/8) bullion of respective grade is now charged into kettle A', so that the kettles A', A<sup>3</sup> and 80 A<sup>5</sup> will be full after the metal in the kettles A<sup>2</sup>, A<sup>4</sup> has been crystallized and the pressed out liquids from kettles A<sup>2</sup> and A<sup>4</sup> tapped into kettles A', A<sup>3</sup> and A<sup>5</sup> from A<sup>2</sup> and A<sup>4</sup>, and melted crystals tapped from 85 kettles A<sup>2</sup> and A<sup>4</sup> into kettles A<sup>3</sup> and A<sup>5</sup>, respectively. Charging with bullion is done from time to time as needed, but the bullion charged into a kettle must be of the respective grade, that is, the same number of 90 ounces of silver per ton, in order to keep the plant in full operation.

From the foregoing it will be seen that by the arrangement described it requires only six operations to produce market lead at 95 one end and five hundred ounces per ton enriched metal at the other end. As is well known, with the processes now in use it requires the employment of about twelve kettles and a corresponding number of crystallization operations to make market lead and enriched metal as above described.

It is understood that I do not limit myself to running the bullion at the seven-eighths (7/8) proportion above explained, as the same 105 process may be carried out on any fraction.

Instead of using mechanical means (plunger K) for pressing out the uncrystallized liquid, use may be made of fluid pressure for the same purpose. In the apparatus 110 shown in Fig. 4, the kettle A<sup>6</sup> is provided with a cover A<sup>7</sup> carrying a valved pipe U connected with a fluid pressure supply such as steam, compressed air or the like, and the kettle is further provided with valved outlets C<sup>2</sup> and K<sup>7</sup>, of which the outlet K<sup>7</sup> is for the discharge of the uncrystallized liquid squeezed out of the crystals by the fluid pressure on top of the mass in the kettle A<sup>6</sup>. A strainer K<sup>8</sup> is arranged in the kettle A<sup>6</sup> 120 over the entrance to the pipe K<sup>7</sup> to prevent the crystals from passing out of the kettle by way of the pipe K<sup>7</sup>, it being understood that the crystals are discharged from the kettle by way of the outlet C<sup>2</sup>.

Although I have shown one particular way of agitating the molten metal in the kettles for effecting crystallization, it is evident that other means may be employed for 125 this purpose, and it is also understood that 130

I do not limit myself to the particular construction of the press H employed, as other mechanical or fluid pressure may be used for carrying on the pressing operation.

5 Having thus described my invention, I claim as new and desire to secure by Letters Patent:

1. The herein described process of refining and desilverizing impure lead, which 10 consists in melting the impure lead bullion, crystallizing a portion of the lead from the molten bullion, separating the molten impure lead from the crystallized lead by pressure applied to the crystals, and conducting 15 the impure lead away from the crystals.

2. The herein described process of refining and desilverizing impure lead bullion, which consists in melting the impure lead bullion, crystallizing a portion of the lead 20 from the molten bullion by cooling and agi-

tation, separating the molten impure lead from the crystallized lead by mechanical pressure applied to the crystals, and conducting the impure lead away from the crystals.

3. The herein described process of refining impure lead which consists in melting the impure lead, crystallizing a portion of the lead from the molten mass, separating the molten impure lead from the crystallized 30 lead by pressure applied to the crystals, and conducting the impure lead away from the crystals.

In testimony whereof I have signed my name to this specification in the presence of 35 two subscribing witnesses.

GEORGE P. HULST.

Witnesses:

THEO. G. HOSTER,

PHILIP D. ROLLHAUS.

Copies of this patent may be obtained for five cents each, by addressing the "Commissioner of Patents, Washington, D. C."